# EUROPEAN PATENT SPECIFICATION

(11) **EP 2 692 884 B1**
(45) Date of publication and mention of the grant of the patent: **03.05.2017**
(21) Application number: 12765196.6
(22) Date of filing: 28.03.2012
(51) Int. Cl.: C22C 23/02, C22F 1/06, C22F 1/00

(54) **MAGNESIUM ALLOY**
MAGNESIUMLEGIERUNG
ALLIAGE DE MAGNÉSIUM

(30) Priority: 29.03.2011 JP 2011072505
(43) Date of publication of application: 05.02.2014
(73) Proprietor: Advanced Technologies, Inc., Gotenba-shi, Shizuoka 412-0047 (JP); Osaka Prefecture University Public Corporation, Osaka 599-8531 (JP)
(72) Inventor: HIRAI, Kinji, Gotenba-shi Shizuoka 412-0047 (JP); HIGASHI, Kenji, Osakasayama-shi Osaka 589-0005 (JP); TAKIGAWA, Yorinobu, Sakai-shi Osaka 599-8531 (JP); UESUGI, Tokuteru, Sakai-shi Osaka 599-8531 (JP)
(74) Representative: Beckmann, Claus
(86) International application number: PCT/JP2012/058113
(87) International publication number: WO 2012/133522

(56) References cited:
- JP-A- 2004 360 042
- JP-A- 2007 113 037
- JP-A- 2010 242 146
- V.RAGHAVAN: 'Al-Ca-Mg-Sr(Aluminum-Calcium- Magnesium-Strontium)' JOURNAL OF PHASE EQUILIBRIA AND DIFFUSION vol. 30, no. 6, December 2009, pages 636 - 637, XP055127414

## Description

### Technical Field

The present invention relates to a magnesium alloy, particularly a magnesium alloy having high strength and high heat resistance, which can be worked into a wrought material such as an extruded or forged material.

### Background Art

It is known that magnesium is the lightest and has the highest specific strength among practical metals. In order to realize reduction in carbon dioxide emission amount due to weight reduction of vehicles, and extension in travelable distance on one charge of electric cars, as measures to cope with global warming, use of a magnesium alloy is expanded in various applications, for example, application of parts which underwent weight reduction using a magnesium alloy.

Usually, parts of the magnesium alloy are formed by a casting or die-casting method.

The reason is as follows. That is, conventional various magnesium alloys can achieve comparatively high room-temperature strength by grain size refinement through plastic working including extrusion, rolling and forging. Meanwhile, since grain boundary precipitates formed into a network undergo fracture, tensile characteristics at high temperature deteriorate, thus leading to limitation of use of a wrought material obtained by plastic working as parts to be used at particularly high temperature.

Patent Document 1 discloses that a magnesium alloy containing 0.1 to 15% by weight of calcium and optionally containing aluminum or zinc in the amount which does not exceed two times the amount of calcium is subjected to plastic working including extrusion and rolling, thereby homogeneously dispersing a crushed intermetallic compound in crystal grains, thus leading to an enhancement in mechanical strength.

Patent Document 2 discloses that refining of crystal grains is suppressed by performing hot rolling or forging at a predetermined processing temperature and rolling reduction ratio using a Mg-Al-Ca-Sr-Mn based alloy, and heat resistance is improved by controlling an aspect ratio of crystal grains (length of a major axis of crystal grains/length of a minor axis of crystal grains) without causing drastic fracture of a network intermetallic compound precipitated in the grain boundary.

Patent Document 3 relates to the problem to provide an Mg-Al-Zn alloy material which has ≥ 300 MPa tensile strength and uniform mechanical properties and can be easily manufactured by extrusion. As a solution to this problem, the document describes an Mg-Al-Zn alloy material which includes: (1) a high strength magnesium alloy extruded material which has a composition consisting of 6 to 15% Al, ≤ 4% Zn and the balance Mg and in which solid-solution Al comprises ≥ 40% of the Al; (2) a high strength magnesium alloy extruded material composed of the above (1), in which the average grain size of crystals constituting the alloy material in the cross-sectional central part is made to ≤ 10 µm; and (3) a high strength magnesium alloy extruded material composed of the above (1) or (2), in which a ratio between the average grain size A of crystals constituting the alloy material in the vicinity of an outer periphery and the average grain size B of crystals constituting the alloy material in the cross-sectional central part satisfies the relation of 1.3 ≥ A/B ≥ 0.7.

### Conventional Art Documents

### Patent Documents

Patent Document 1: JP 2000-109963 A
Patent Document 2: JP 2007-70688 A
Patent Document 3: JP 2007-113037 A

### Disclosure of the Invention

### Problems to be Solved by the invention

However, the magnesium alloy according to Patent Document 1 had a problem that it is still insufficient in heat resistance, i.e. strength at high temperature.

Meanwhile, the magnesium alloy according to Patent Document 2 had a problem that it is necessary to suppress the working degree (rolling reduction ratio) of hot rolling and forging to a low value so as to obtain a defined aspect ratio of crystal grains, so that the strength at room temperature may be sometimes insufficient.

Thus, the magnesium alloys of Patent Documents 1 and 2 may be sometimes insufficient in high-temperature strength or room-temperature strength.

Even in the case of a magnesium alloy used at high temperature, the environmental temperature necessarily includes a range from room temperature to high temperature. Therefore, it is necessary that tensile characteristics of the magnesium alloy are excellent in both environments at room temperature and high temperature in practical use. Accordingly, a magnesium alloy having sufficient strength at room temperature and high temperature has been required.

The present invention has been made so as to meet the requirements, and thus an object thereof is to provide a magnesium alloy which has sufficiently high strength at room temperature and high temperature.

### Means for Solving the Problems

A first aspect of the present invention is directed to a magnesium alloy including: aluminum (Al): 14.0 to 23.0% by mass, calcium (Ca) : 11.0% by mass or less (not including 0% by mass), strontium (Sr): 12.0% by mass or less (not including 0% by mass), and zinc (Zn): 0.2 to 1.0% by mass, and the balance magnesium (Mg) and inevitable impurities, wherein the content of aluminum (A1), the content of calcium (Ca), and the content of strontium (Sr) satisfy a relation shown in the following equation (1): $0.8 \times < Al > \leq 1.35 \times < Ca > + 1.23 \times < Sr > + 8.5 \leq 1.2 \times < Al >$ where <A1> is the content of aluminum (Al) expressed on % by mass basis, <Ca> is the content of calcium (Ca) expressed on % by mass basis, and <Sr> is the content of strontium (Sr) expressed on % by mass basis.

A second aspect of the present invention is directed to the magnesium alloy according to the first aspect, further including at least one selected from the group consisting of silicon (Si): 0.1 to 1.5% by mass, rare earth (RE): 0.1 to 1.2% by mass, zirconium (Zr): 0.2 to 0.8% by mass, scandium (Sc): 0.2 to 3.0% by mass, yttrium (Y): 0.2 to 3.0 % by mass, tin (Sn): 0.2 to 3.0% by mass, barium (Ba): 0.2 to 3.0% by mass, and antimony (Sb): 0.1 to 1.5% by mass.

A third aspect of the present invention is the magnesium alloy according to the first or second aspect, in which a ratio of the content of strontium (Sr) to the content of calcium (Ca) is from 1:0.3 to 1:1.5 in terms of a mass ratio.

A fourth aspect of the present invention is directed to the magnesium alloy according to any one of the first to third aspects, in which precipitates containing Al₂Ca and Al₄Sr are formed in the grain boundary with an interval from each other.

### Effects of the Invention

According to the present invention, it is made possible to provide a magnesium alloy having sufficient room-temperature strength and sufficient high-temperature strength.

### Brief Description of the Drawings

Figs. 1A to 1C show metallographic structures observed by a confocal laser scanning microscope, in which Fig. 1A shows a metallographic structure of an as-extruded material, Fig. 1B shows a metallographic structure of a material subjected to a homogenization heat treatment at 400°C for 48 hours, and Fig. 1C shows a metallographic structure of a material subjected to a homogenization heat treatment at 420°C for 48 hours.
Fig. 2 shows the results of a high-temperature tensile test at 150°C (true stress-strain diagram) of an as-extruded material, a material subjected to a homogenization heat treatment at 400°C for 48 hours, and a material subjected to a homogenization heat treatment at 420°C for 48 hours.
Fig. 3 shows the measurement results of a tensile strength at room temperature.
Fig. 4 shows the measurement results of a tensile strength at high temperature.

### Embodiments for Carrying Out the Invention

The present inventors have made a study on simultaneous utilization of both solid solution strengthening and precipitation strengthening known as strengthening mechanisms of a magnesium alloy.

That is, they have made a study on effective actuation of both solid solution strengthening mechanism and precipitation strengthening mechanism by appropriate control of the contents of aluminum, strontium and calcium.

Subsequently, the present inventors have determined solid solubility limit of aluminum in a magnesium alloy matrix and found appropriate amounts of aluminum, calcium and strontium on the basis of the solid solubility limit, and thus completing a magnesium alloy according to the present invention, having sufficient strength at both room temperature and high temperature in which a matrix forms a solid solution with a sufficient amount of aluminum, and also an appropriate amount of intermetallic compounds Al₂Ca and Al₄Sr are precipitated.

Detailed description will be made below.

### (1) Aluminum

In the deformation at high temperature of the magnesium alloy, low stacking fault energy suppresses the movement of dislocations, resulting in the difficulty in deformation. Thus, if stacking fault energy can be lowered, heat resistance (high-temperature strength and creep) can be improved.

Examples of the element capable of being solid-soluted in a magnesium alloy to lower stacking fault energy include In, Tl, Sc, Pb, Al, Y, Sn and Bi. Of these elements, aluminum (Al) is preferable from the viewpoint of safety and economy.

As a result of the present inventors' study, it has been found the addition of calcium (Ca) and strontium (Sr), together with aluminum, enables refining of the grain size, leading to an enhancement in room-temperature strength, and also intermetallic compounds Al₂Ca and Al₄Sr to be precipitated (crystallized) exist in the grain boundary, together with other second phases (precipitates), thereby improving room temperature and high temperature characteristics.

If the magnesium alloy is worked into a wrought material by performing plastic working including rolling, extrusion and drawing after casting so as to obtain desired shape, toughness, strength and the like, second phases containing Al₂Ca and Al₄Sr precipitating in the grain boundary are fractured (fragmented) and arranged in the deformation direction.

The precipitates containing Al₂Ca and Al₄Sr thus arranged in the deformation direction contribute to an enhancement in high-temperature strength.

However, the present inventors have intensively studied and found that second phase particles containing Al₂Ca and Al₄Sr can be reprecipitated and dispersed by performing a homogenization heat treatment at 350 to 450°C, leading to more enhancement in strength. It has also been found that, more preferably, second phases containing Al₂Ca and Al₄Sr can be homogeneously dispersed in the grain boundary by performing a homogenization heat treatment at 385°C to 415°C, and thus enabling an increase in strength more certainly.

As a result of the continued study, the present inventors have found that maximum solubility (solid solubility limit) of aluminum in matrix of the sample subjected to a homogenization heat treatment at 400°C for 48 hours after plastic working such as extrusion is 8.3% by mass (7.5 atomic %). The measurement was performed by point analysis using an electron probe microanalyzer (EPMA).

Using this solid solubility limit, the present inventors have found that the amount of aluminum of the magnesium alloy according to the present invention is appropriately from 14.0 to 23.0% by mass.

The reason is that, if the amount of aluminum is 14.0% by mass or more, a sufficient amount of aluminum can form intermetallic compounds Al₂Ca and Al₄Sr with calcium and strontium even if about 8.5% by mass of aluminum is solid-soluted in the matrix. If the amount of aluminum is 23.0% by mass or less, it is possible to ensure ductility such as elongation.

More preferably, the amount of aluminum is from 15.0% by mass to 20.0% by mass.

This is because it is possible to form intermetallic compounds Al₂Ca and Al₄Sr more certainly and to ensure ductility if the amount of aluminum is within the above range.

### (2) Calcium

The content of calcium is 11.0% by mass or less (not including 0% by mass).

The maximum content (11.0% by mass) of calcium is almost equal to the amount of calcium required for almost all aluminum, which was not solid-soluted, to form Al₂Ca ((upper limit of aluminum - maximum solubility)/atomic weight of Al × atomic ratio of Ca to Al of Al₂Ca × atomic weight of Ca = 10.9). Thus, it is made possible to certainly precipitate aluminum, which is not solid-soluted, as a desired intermetallic compound.

In order to ensure inclusion of calcium, 0% by mass is excluded.

More preferably, the content of calcium is from 1.0 to 8.0% by mass. This is because it is possible to form Al₂Ca more certainly and to suppress excessiveness.

### (3) Strontium

The content of strontium is 12.0% by mass or less (not including 0% by mass).

The maximum content (12.0% by mass) of strontium is almost equal to the amount of calcium required for almost all aluminum, which was not solid-soluted, to form Al₄Sr ((upper limit of aluminum - maximum solubility)/atomic weight of Al ×atomic ratio of Sr to Al of Al₄Sr × atomic weight of Sr = 11.9). Thus, it is made possible to certainly precipitate aluminum, which is not solid-soluted, as a desired intermetallic compound.

In order to ensure inclusion of strontium, 0% by mass is excluded.

Preferably, the content of strontium is from 0.5 to 8.0% by mass. This is because it is possible to form Al₄Sr more certainly and to suppress excessiveness. More preferably, the content is from 1.0 to 6.0% by mass. This is because it is possible to maximally exert the effect of strontium.

### (4) Zinc

The magnesium alloy according to the present invention contains 0.2 to 1.0% by mass of zinc (Zn).

This is because zinc has the effect of enhancing the strength and the effect of improving castability.

### (5) Relation among Aluminum, Calcium and Strontium

### - Ratio of Calcium to Strontium

In order to form both intermetallic compounds Al₂Ca and Al₄Sr in a more suitable ratio (ratio of formation amount of Al₂Ca and Al₄Sr), a ratio of (content of calcium):(content of strontium) (content of strontium assumed that the content of calcium is 1) is preferably from 1:0.3 to 1:1.5 in terms of a mass ratio, and more preferably 1:0.5 to 1:1.1 in terms of a mass ratio.

### - Relation among Aluminum Content, Calcium Content and Strontium Content

In the magnesium alloy according to the present invention, in order to enable entire strontium and calcium to precipitate as Al₂Ca and Al₄Sr, respectively, the amount of aluminum (% by mass) indicated by the symbol y in the equation (2) is required.$y = < Ca > / 40.08 \left(atomic weight of Ca\right) \times 2 \left({atomic ratio of Al to Ca of Al}_{2}Ca\right) \times 26.98 \left(atomic weight of Al\right) + < Sr > / 87.62 \left(atomic weight of Sr\right) \times 4 \left({atomic ratio of Al to Sr of Al}_{4}Sr\right) \times 26.98 \left(atomic weight of Al\right) + 8.3 \left(maximum solubility of Al\right) = 1.35 \times < Ca > + 1.23 \times < Sr > + 8.5$

In this equation, <Ca> is the content of calcium expressed on % by mass basis and <Sr> is the content of strontium expressed on % by mass basis.

Physical meaning of a numerical value in the equation is shown in parentheses behind the numerical value.

In the magnesium alloy according to the present invention, it is necessary to satisfy the following equation (1).

That is, aluminum is contained such that the amount of aluminum (y) represented by the equation (2), which is required for entire strontium and calcium to precipitate as Al₂Ca and Al₄Sr, respectively, is within a range of the amount which is 0.8 to 1.2 times the content of aluminum.

This is because, when the content of aluminum is within a range represented by the equation (1), Al₂Ca and Al₄Sr, which are almost equal to the stoichiometric composition, are precipitated and also aluminum is sufficiently solid-soluted in the matrix in just proportion of all elements of aluminum, calcium and strontium.$0.8 \times < Al > \leq 1.35 \times < Ca > + 1.23 \times < Sr > + 8.5 \leq 1.2 \times < Al >$ where <Al> is the content of aluminum expressed on % by mass basis.

### (6) Other Components

The alloy of the present invention contains the above-mentioned aluminum, calcium, strontium and zinc, with the balance being magnesium (Mg) and inevitable impurities.

### (7) Heat Treatment

Al₂Ca and Al₄Sr are often precipitated in the grain boundary, as second phases containing Al₂Ca and Al₄Sr, in the form of a network. As mentioned above, when subjected to plastic working, the second phases containing network Al₂Ca and Al₄Sr (precipitates) tend to be fractured (fragmented) and arranged in the deformation direction.

Since the thus fragmented precipitates containing Al₂Ca and Al₄Sr contribute to an improvement in high-temperature strength, a magnesium alloy article (magnesium alloy wrought material) obtained by plastic working (plastic deformation) also has high-temperature strength.

However, second phase particles containing Al₂Ca and Al₄Sr can be reprecipitated and dispersed by performing a homogenization heat treatment at 350 to 450°C after plastic working, thereby finding that high-temperature strength can be more enhanced. Therefore, the magnesium alloy according to the present invention (magnesium alloy article (wrought material)) is preferably subjected to a homogenization heat treatment at 350 to 450°C after plastic working. In the homogenization heat treatment at 350 to 450°C, it is preferred to maintain within such temperature range for 24 to 72 hours. This is because this treatment enables redissolution (reprecipitation) of precipitates, leading to an improvement in heat stability.

The present inventors have also found that a homogenization heat treatment at 385°C to 415°C enables reprecipitation of second phase particles containing Al₂Ca and Al₄Sr and homogeneous dispersion of the second phase particles along the grain boundary, leading to further improvement in high-temperature strength. In case a homogenization treatment is performed at 385°C to 415°C after plastic working, second phase particles containing Al₂Ca and Al₄Sr (precipitates) are precipitated in the form of particles, instead of a network, with an interval from each other (i.e. discontinuously) along the grain boundary. The thus obtained precipitates in this form remarkably contribute to an improvement in high-temperature strength. Therefore, the magnesium alloy according to the present invention (magnesium alloy article (wrought material)) is preferably subjected to a homogenization heat treatment at 385 to 415°C after plastic working. In the homogenization heat treatment at 385 to 415°C, it is preferred to maintain within such temperature range for 24 to 72 hours. This is because this treatment enables redissolution of precipitates and homogenization of the structure, leading to homogenization and stabilization of an intermetallic compound structure with high heat stability of the grain boundary.

As used herein, plastic working includes various hot and cold plastic workings. Examples of the plastic working include extrusion, rolling, forging, drawing, swaging, and combinations thereof.

### Examples

Alloy samples, each containing components shown in Table 1, were prepared.

The value y in the equation (2) of samples of Examples (Example 1 and Example 2) shown in Table 1 is 15.5 in Example 1 and is 20.9 in Example, and therefore alloy samples satisfy the equation (1). In both Example 1 and Example 2, a ratio of (content of calcium):(content of strontium) is 1:1 in terms of a mass ratio.

**Table 1**

| | Comparative Example 1 | | Example 1 | | Example 2 | | Comparative Example 2 | | Comparative Example 3 | |
|---|---|---|---|---|---|---|---|---|---|---|
| | Mass % | Atomic % | Mass % | Atomic % | Mass % | Atomic % | Mass % | Atomic % | Mass % | Atomic % |
| Mg | 88.1 | 90.0 | 79.1 | 80.8 | 69.9 | 71.4 | 60.9 | 62.2 | 51.9 | 53.0 |
| Al | 10.0 | 9.2 | 15.0 | 13.8 | 20.0 | 18.4 | 25.0 | 23.0 | 30.0 | 27.6 |
| Ca | 0.7 | 0.4 | 2.7 | 1.7 | 4.8 | 3.0 | 6.8 | 4.2 | 8.8 | 5.5 |
| Sr | 0.7 | 0.2 | 2.7 | 0.8 | 4.8 | 1.4 | 6.8 | 1.9 | 8.8 | 2.5 |
| Zn | 0.5 | 0.2 | 0.5 | 0.2 | 0.5 | 0.2 | 0.5 | 0.2 | 0.5 | 0.2 |

Each alloy sample was melted at 700°C and then cast into a billet using a cylindrical die. The casted billet was heated to 400°C at a heating rate of 0.5°C/minute, maintained for 48 hours and then water-cooled. After removing a surface oxide layer by machining, the billet was extruded at an extrusion temperature of 350°C, an extrusion rate of 0.2 mm/second and an extrusion ratio of 16 to obtain a round bar (10 mm in diameter).

### 1) Homogenization Heat Treatment

In order to examine an influence of a homogenization heat treatment, regarding the above-mentioned sample of Example 1 (extruded round bar), an as-extruded material, a material subjected to a homogenization heat treatment at 400°C for 48 hours, and a material subjected to a homogenization heat treatment at 420°C for 48 hours were produced.

Figs. 1A to 1C show metallographic structures observed by a confocal laser scanning microscope, in which Fig. 1A shows a metallographic structure of an as-extruded material, Fig. 1B shows a metallographic structure of a material subjected to a homogenization heat treatment at 400°C for 48 hours, and Fig. 1C shows a metallographic structure of a material subjected to a homogenization heat treatment at 420°C for 48 hours.

In the as-extruded material, precipitates containing Al₂Ca and Al₄Sr (second phases) are fragmented and arranged in the extrusion direction (up/down direction in the drawing). In contrast, in the material subjected to a homogenization heat treatment at 400°C for 48 hours and the material subjected to a homogenization heat treatment at 420°C for 48 hours, precipitates containing Al₂Ca and Al₄Sr (second phases) are dispersed. Particularly in the material subjected to a homogenization heat treatment at 400°C for 48 hours, granular precipitates containing comparatively fine Al₂Ca and Al₄Sr are homogeneously distributed with an interval from each other along the grain boundary.

Fig. 2 shows the results of a high-temperature tensile test at 150°C (true stress-strain diagram) of an as-extruded material, a material subjected to a homogenization heat treatment at 400°C for 48 hours, and a material subjected to a homogenization heat treatment at 420°C for 48 hours. The tensile test was carried out at a temperature of 150°C and a tension speed of 1 × 10⁻³/second.

All samples exhibit excellent high-temperature strength (heat resistance), that is, tensile strength at 150°C of 250 MPa. Of these, the material subjected to a homogenization heat treatment at 400°C for 48 hours and the material subjected to a homogenization heat treatment at 420°C for 48 hours exhibit high-temperature strength which is higher than that of the as-extruded material. Particularly, the material subjected to a homogenization heat treatment at 400°C for 48 hours has high-temperature strength which is remarkably high strength of more than 300 MPa.

Considering the above results, subsequent evaluation was carried out after homogenizing the extruded round bars of Examples 1 and 2 as well as Comparative Examples 1 to 3 at 400°C for 48 hours and processing them into tensile test specimens.

### 2) Measurement Results of Grain Size

The grain size of each alloy sample is shown in Table 2.

The grain size was measured by the electron back scattered diffraction patterns (EBSD) method. Crystal grains were defined by regarding deviation of orientation of 15° or more as the grain boundary.

The average grain size was determined by simply dividing the total area by the number of crystal grains.

**Table 2**

| Alloy | Grain size (µm) |
|---|---|
| Comparative Example 1 | 20.1 |
| Example 1 | 9.2 |
| Example 2 | 4.9 |
| Comparative Example 2 | 4.2 |
| Comparative Example 3 | - |

In Comparative Example 3, the grain size could not be measured since precipitates underwent coarsening. Except for Comparative Example 3, the grain size (both peak-top grain size and area average particle size) decreases as addition amounts of aluminum, calcium and strontium increases.

### 3) Room-Temperature Tensile Characteristics

Fig. 3 shows the measurement results of the tensile strength at room temperature. The drawing shows the measurement results of the tensile strength, 0.2% proof stress, and elongation of each alloy sample. In Comparative Examples 2 and 3, 0.2% proof stress could not be measured since the material is brittle.

In Comparative Example 1, Example 1 and Example 2, the tensile strength exhibited excellent value such as 300 MPa or more. However, it is apparent that, in Comparative Example 1, the 0.2% proof stress is less than 250 MPa, and the samples of Example 1 and Example 2 having the 0.2% proof stress of 250 MPa or more are excellent in room-temperature strength as compared with the samples of Comparative Examples. It is also apparent that the samples of Example 1 and Example 2 exhibit the elongation of 2% or more and have sufficient ductility.

It is also known that the sample, which is produced by extruding an AZ91 alloy known as a high strength magnesium alloy at an extrusion temperature of 360°C and an extrusion ratio of 22, each being the same level as that of the samples of Examples 1 and 2, exhibits the tensile strength of 295 MPa (Hanlin Ding et al., Journal of alloys and compounds, 456(2008) 400-406). As is apparent from these results, the samples of Examples 1 and 2 have high room-temperature strength.

### 4) High-Temperature Strength

Fig. 4 shows the measurement results of high-temperature tensile strength. The high-temperature tensile test was carried out at a measuring temperature of 175°C and a strain rate of 1 × 10⁻⁴/second.

Since the sample of Comparative Example 3 was fractured soon after applying tensile stress, high-temperature strength could not be measured.

The samples of Example 1 and Example 2 exhibited high-temperature strength which is higher than that in Comparative Examples, that is, high-temperature strength at 175°C is 210 MPa or more.

As is apparent from the above results, the samples of Examples exhibit high strength at both room temperature and high temperature.

## Claims

1. A magnesium alloy comprising:
aluminum (Al): 14.0 to 23.0% by mass,
calcium (Ca): 11.0% by mass or less (not including 0% by mass),
strontium (Sr): 12.0% by mass or less (not including 0% by mass),
zinc (Zn): 0.2 to 1.0% by mass, and optionally Si, RE, Zr, Sc, Y, Sn, Ba, Sb,
the balance magnesium (Mg) and inevitable impurities, wherein the content of aluminum (Al), the content of calcium (Ca), and the content of strontium (Sr) satisfy a relation shown in the following equation (1): $0.8 \times < Al > \leq 1.35 \times < Ca > + 1.23 \times < Sr > + 8.5 \leq 1.2 \times < Al >$ where <Al> is the content of aluminum (Al) expressed on % by mass basis, <Ca> is the content of calcium (Ca) expressed on % by mass basis, and <Sr> is the content of strontium (Sr) expressed on % by mass basis.

2. The magnesium alloy according to claim 1, further comprising at least one selected from the group consisting of:
silicon (Si): 0.1 to 1.5% by mass,
rare earth (RE): 0.1 to 1.2% by mass,
zirconium (Zr): 0.2 to 0.8% by mass,
scandium (Sc): 0.2 to 3.0% by mass,
yttrium (Y): 0.2 to 3.0 % by mass,
tin (Sn): 0.2 to 3.0% by mass,
barium (Ba): 0.2 to 3.0% by mass, and
antimony (Sb): 0.1 to 1.5% by mass.

3. The magnesium alloy a ccording to claim 1 or 2, wherein a ratio of the content of strontium (Sr) to the content of calcium (Ca) is from 1:0.3 to 1:1.5 in terms of a mass ratio.

4. The magnesium alloy according to any one of claims 1 to 3, wherein precipitates containing Al₂Ca and Al₄Sr are formed in the grain boundary with an interval from each other.

## Patentansprüche

1. Magnesiumlegierung, umfassend:
Aluminium (Al): 14,0 bis 23,0 Massen-%,
Calcium (Ca): 11,0 Massen-% oder weniger (ausschließlich 0 Massen-%),
Strontium (Sr): 12,0 Massen-% oder weniger (ausschließlich 0 Massen-%),
Zink (Zn): 0,2 bis 1,0 Massen-%, und gegebenenfalls Si, RE, Zr, Sc, Y, Sn, Ba, Sb,
den Rest Magnesium (Mg) und unvermeidbare Verunreinigungen, wobei der Gehalt an Aluminium (Al), der Gehalt an Calcium (Ca) sowie der Gehalt an Strontium (Sr) der in der folgenden Gleichung (1) gezeigten Beziehung genügen: $0 , 8 \times < Al > \leq 1 , 35 \times < Ca > + 1 , 23 \times < Sr > + 8 , 5 \leq 1 , 2 \times < Al >$ wobei <Al> der Gehalt an Aluminium (Al) ist, ausgedrückt auf Massenprozentbasis, <Ca> der Gehalt an Calcium (Ca) ist, ausgedrückt auf Massenprozentbasis und <Sr> der Gehalt an Strontium (Sr) ist, ausgedrückt auf Massenprozentbasis.

2. Magnesiumlegierung gemäß Anspruch 1, des Weiteren umfassend wenigstens eines, ausgewählt aus der Gruppe, bestehend aus:
Silicium (Si): 0,1 bis 1,5 Massen-%,
seltene Erden (RE): 0,1 bis 1,2 Massen-%,
Zirkonium (Zr): 0,2 bis 0,8 Massen-%,
Scandium (Sc): 0,2 bis 3,0 Massen-%,
Yttrium (Y): 0,2 bis 3,0 Massen-%,
Zinn (Sn): 0,2 bis 3,0 Massen-%,
Barium (Ba): 0,2 bis 3,0 Massen-% und
Antimon (Sb): 0,1 bis 1,5 Massen-%.

3. Magnesiumlegierung gemäß Anspruch 1 oder 2, wobei das Verhältnis des Gehalts an Strontium (Sr) zu dem Gehalt an Calcium (Ca) von 1:0,3 bis 1:1,5 als Massenverhältnis reicht.

4. Magnesiumlegierung gemäß einem der Ansprüche 1 bis 3, wobei Präzipitate, welche Al₂Ca und Al₄Sr enthalten, an der Korngrenze mit einem Abstand voneinander gebildet sind.

## Revendications

1. Alliage de magnésium comprenant :
aluminium (Al) : 14,0 à 23,0 % en masse,
calcium (Ca) : 11,0 % en masse ou moins (à l'exclusion de 0 % en masse),
strontium (Sr) : 12,0 % en masse ou moins (à l'exclusion de 0 % en masse),
zinc (Zn) : 0,2 à 1,0 % en masse, et facultativement du Si, RE, Zr, Sc, Y, Sn, Ba, Sb,
le reste étant du magnésium (Mg) et des impuretés inévitables, dans lequel la teneur en aluminium (Al), la teneur en calcium (Ca), et la teneur en strontium (Sr) satisfont à une relation présentée dans l'équation suivante (1) : $0 , 8 \times < Al > \leq 1 , 35 \times < Ca > + 1 , 23 \times < Sr > + 8 , 5 \leq 1 , 2 \times < Al >$ dans laquelle <A1> est la teneur en aluminium (Al) exprimée sur la base du % en masse, <Ca> est la teneur en calcium (Ca) exprimée sur la base du % en masse, et <Sr> est la teneur en strontium (Sr) exprimée sur la base du % en masse.

2. Alliage de magnésium selon la revendication 1, comprenant en outre au moins un élément sélectionné dans le groupe constitué de :
silicium (Si) : 0,1 à 1,5 % en masse,
terres rares (RE) : 0,1 à 1,2 % en masse,
zirconium (Zr) : 0,2 à 0,8 % en masse,
scandium (Sc) 0,2 à 3,0 % en masse,
yttrium (Y) : 0,2 à 3,0 % en masse,
étain (Sn) : 0,2 à 3,0 % en masse,
baryum (Ba) : 0,2 à 3,0 % en masse, et
antimoine (Sb) : 0,1 à 1,5 % en masse.

3. Alliage de magnésium selon la revendication 1 ou 2, dans lequel un rapport du contenu de strontium (Sr) sur le contenu de calcium (Ca) est de 1/0,3 à 1/1,5 en termes d'un rapport en masse.

4. Alliage de magnésium selon l'une quelconque des revendications 1 à 3, dans lequel des précipités contenant de l'Al₂Ca et de l'Al₄Sr sont formés dans l'interface cristalline avec un intervalle entre eux.
